

Sept. 27, 1927.

1,643,333

E. E. CHANDLER

METHOD OF MEASURING THE STRENGTH OF FIBERS

Filed May 7, 1925



Fig. 1.



Fig. 2.

Fig. 3.



Elbert E Chandler INVENTOR.

## UNITED STATES PATENT OFFICE.

ELBERT E. CHANDLER, OF LOS ANGELES, CALIFORNIA.

## METHOD OF MEASURING THE STRENGTH OF FIBERS.

Application filed May 7, 1925. Serial No. 28,697.

My invention relates particularly to cotton fiber, although it may be applied to hairs, filaments and other fibers, such as are used mainly in textiles. It consists in the preparation of a bundle of such fibers, the measurement of the superficial cross sectional area of the bundle, the reduction of this superficial area to the area of the material tested, with elimination of the interstices or voids, the preparation of the bundle for unit breakage, the final breakage of the bundle and the calculation of the strength of the material compassing it.

Present methods of testing small fibers consist of breaking single fibers to determine their strength. In a test recently made the strength of a series of one hundred fibers of cotton taken at random was found to vary from two grams to 14.5 grams so that little reliability can be placed on this method without a large number of tedious operations. Other methods such as twisting together a certain weight of fibers and breaking them and also breaking a number of parallel fibers whose ends had been pasted to a card board and the cardboard slit into two portions, so that the strain came entirely on the fibers, have been tried. These methods however do not give the strength of the cellulose, but merely the average strength of the fiber. They are also subject to a number of other limitations and have found no practical use.

The bundle of fibers is prepared in a manner similar to that used by the cotton stapler, when he estimate the length of the fiber. I prefer however to further even up the bundle or "pull" by combing it at successive stages through a stationary comb. This makes the fiber more parallel and removes motes and tangles, which it is impossible to entirely remove by hand.

The bundle is then wrapped with thread by means of the machine illustrated in the accompanying drawing in which Figure 1 represents a top view of the wrapping device, Figure 2 a front elevation and Figure 3 a bundle of cotton to whose ends a thread has been tied and which is ready to be wrapped. To do so it is clamped in the jaws  $a$  and  $a'$ . The bundle  $b$  is then stretched by the weight  $c$ , suspended by the string  $d$ , running over the pulley  $e$  from the swivel  $f$ , attached to the shaft  $g$ , integral with the jaw  $a$ . The jaw  $a$  is made to ro-

tate with the jaw  $a'$  by means of the gears  $h$ ,  $h'$ ,  $h''$  and  $h'''$  and the jack shaft  $i$ , when the shaft  $g$  is rotated by the crank  $j$ .

The thread  $k$  is thus wrapped on the bundle, while being stretched by the second weight  $l$ . Weights  $l$  and  $c$  of one and two pounds, two and five and four and ten pounds respectively have been tried and a number 20 thread has been found sufficient to suspend the smaller or wrapping weight. The greater the weight on the wrapping thread the greater the degree of condensation of the fibers or the elimination of the interstices between them. Slightly greater condensation results also when the bundles have been wet with alcohol, rinsed with water and wrapped while still wet or after drying. All of these cases have been investigated and the most suitable methods chosen.

The following formulæ are used in calculating the strength of the cellulose enclosed by the thread. Let the strength in pounds per square inch of cross section be represented by  $S$ , the break in pounds of the bundle by  $B$ , the diameter and circumference of the bundle by  $D$  and  $C$  respectively, and the constant by which to multiply the result in order to eliminate the voids by  $K$ , then;

$$A_1 = \frac{\pi D^2}{4}; D^2 = \frac{C^2}{\pi^2}; A_1 = \frac{C^2}{4\pi}; S = \frac{KB}{A_1} = \frac{4KIB}{C^2}.$$

The cellulose strength  $S$  may also be found more directly if the length of the bundle is known. However the fibers in the bundle are of varying lengths and this length of the bundle can not be determined by direct measurement. A method has been devised to determine this average cellulose length and, if the weight of the bundle be represented by  $W$ , the density of cellulose or other material by  $D_e$ , the volume by  $V$ , its area by  $A$  and the average length by  $L$ , then;

$$V = \frac{W}{D_e}; A_2 = \frac{V}{L}; D_eL = \frac{BDeL}{W}.$$

The value of  $K$  is merely the ratio of the areas  $A_1$  and  $A_2$  obtained by the two methods, or;

$$K = \frac{A_1}{A_2} = \frac{\frac{C^2}{4\pi}}{\frac{BDeL}{W}} = \frac{C^2 DeL}{4\pi W}.$$

To obtain the value of  $K$ ,  $L$  may be made short enough to include all the fibers. This

was done by placing the wrapped bundle under a straight edge three eighths of an inch wide and pressing upon it with a sharp knife.

5 The density of cellulose in the metric system is usually given as 1.5. The three eighths inch bundle was dried, unwrapped and weighed in grams. Converting all terms to the English system of units

10

$$K = .733 \frac{C^2}{W}$$

and the values of K were found at the various tensions and conditions investigated. At 15 two and five pound tensions, wetting the cotton and allowing it to dry to standard conditions this constant K was found to be 1.76, whereas when the cotton was wrapped wet the K became 1.64. When wrapped at 20 four and ten pound tensions K, when cotton had never been wet, was 1.62, when wet and allowed to dry 1.56 and when wrapped wet 1.61. When the bundle had never been wet and the value of K was 1.62 the formula for 25 the strength of the cellulose of cotton fiber in pounds per square inch became substantially

30

$$20 \frac{B}{C^2}$$

The bundles were wrapped from ends to middle. When the thread windings met they reversed their direction and moved to the ends. This left a place in the middle of the 35 bundle which was supported by the fiber alone when stressed in the breaker jaws. The position of the indicator on the scale  $n$  was noted when the wrappings were about three eighths of an inch apart and then again after 40 ten revolutions of the crank. This allowed an easy calculation of the denominator of the last equation. The break was made on the ordinary yarn breaker, although special jaws had to be constructed to hold the 45 bundle. 10,000 fibers were found to have a

circumference of about .16 inches and to break at about 100 pounds. Bundles from half this number to three times this number were found to give good agreement for the strength of cellulose by this formula. No account need be taken for the thickness of the wrapping thread as the circumference occurs in the numerator in determining the value of K and in the denominator in determining the value of S. The cellulose of 55 different cottons was found to vary considerably, running from 100,000 pounds to the square inch to about half that amount. The results by this method were compared with those by the single fiber method and found 60 to be in good agreement, without the seven hundred per cent difference exhibited by single fibers. The probable error by this method is less than 2 per cent.

While wrapping a round body is a well 65 known method of obtaining its area, yet it is done here not only for this purpose but also to prepare the bundle to give a sharp snappy break. This break always occurs where the wrappings have met and resistance 70 can only be due to the fibers. Other methods of wrapping have been tried, such as for instance wrapping only in one direction. This gives a slightly greater strength to the bundle, but the question arises whether some 75 of the apparent strength is not due to the thread, even though the thread is not broken and runs transverse to the fiber.

Having thus described my invention what I claim and desire to secure by Letters Patent, is:—

A method of measuring the strength of fibers, consisting in laying them parallel with each other, wrapping them with a thread to obtain the superficial area of the 85 bundle and to prepare it for an even break and breaking the bundle to obtain its strength.

ELBERT E. CHANDLER.